

## UNITED STATES PATENT OFFICE.

GEORGE R. RICH, OF BATTLE CREEK, MICHIGAN.

## HEAT-RESISTING ALLOY STEEL AND ARTICLES MADE THEREFROM.

No Drawing.

Application filed April 27, 1925. Serial No. 26,296.

To all whom it may concern:

Be it known that I, GEORGE R. RICH, a citizen of the United States, and a resident of Battle Creek, Calhoun County, and State of Michigan, have invented certain new and useful Improvements in Heat-Resisting Alloy Steel and Articles Made Therefrom, of which the following is declared to be a full, clear, and exact description.

10 This invention relates to heat resisting alloy steel and articles made therefrom, in which the property of being non-scaling or resistant to hot oxidation when heated to high temperature, is of great importance, 15 as for instance when used for poppet valves for internal combustion engines.

The principal object of this invention is to produce an alloy steel in which the conversion is relatively high, and in which the 20 characteristics of the steel obtained from all of the heats will remain substantially constant, whereby the same or substantially the same heat treatment may be used in the production of articles made from the alloy.

25 Many attempts have been made heretofore, to produce an alloy steel suitable for the production of poppet valves, with partial success, but when an attempt has been made to produce a relatively inexpensive alloy 30 steel which will resist hot oxidation, it has been found in the actual manufacture of valves from such steel, that it is "wild"—that is to say, no two heats are alike and consequently one lot of steel requires heat 35 treatment different from another lot and as a result much time, labor and loss of material is experienced in the actual manufacture of valves from such steel. Moreover the conversion is low, sometimes as low 40 as 60 per cent, which as a matter of fact, increases the cost of production of the steel and articles made therefrom.

In accordance with the present invention, alloy steel, containing the materials in and about the proportions specified, runs substantially constant, each heat being practically like the preceding ones; the conversion is relatively high, consequently, while more suitable and desirable materials are used, the cost of production is not so great because the loss in conversion is less. The heads of valves when forged or shaped up by the hammering process will be found to have a smooth, unbroken surface, free from

scale, and requiring no machining. This is 55 a great saving in the cost of production, and by reason of this characteristic of the surface, the valve effectively resists hot oxidation.

The principal alloying elements in the present steel are chromium and nickel; some manganese and silicon are used, and a small quantity of phosphorus and sulphur is present as usual, the remainder is principally iron. The carbon content is relatively low. 60

The proportions may vary slightly within the limits given, and a less efficient alloy may be obtained if some of the materials exceed the specified limits. For obtaining the best results, the following proportions 70 have been used successfully in the manufacture of poppet valves in great numbers:

|                        | Per cent.       |
|------------------------|-----------------|
| Chromium               | 7.00 to 8.00 75 |
| Nickel                 | 1.25 to 2.25    |
| Phosphorus and sulphur | under .03       |
| Manganese              | .45 to .65      |
| Silicon                | .50 to 1.00     |
| Carbon                 | .35 to .45 80   |

The remainder iron.

Valves made from alloy steel containing the materials in the proportions specified in the above schedules are tough and hard and the 85 surface will stand wear and resist hot oxidation. The danger of surface decarbonization, if left in the fire too long, is reduced to a minimum—that is, one of the drawbacks of medium priced alloy steels now on the market for use in the manufacture of valves. The steel is readily workable at temperatures ranging from 1600 to 1800 degrees Fahrenheit, and may be air cooled or quenched in water. The steel is not "wild" 90 but its characteristics remain substantially constant. For this reason the mills are able to produce a medium priced alloy steel which does contain the non-corroding, non-oxidizing characteristics attributed to many of the 100 so called alloys having high resistance to hot oxidation.

I claim as new and desire to secure by Letters Patent:

1. An alloy steel having high resistance to hot oxidation, having a composition substantially as follows: chromium 7.00 to 8.00%; nickel 1.25 to 2.25%; phosphorus and

sulphur together, under .03%; manganese .45 to .65%; silicon .50 to 1.00%; carbon .35 to .45% and the principal part of the remainder iron. 8.00%; nickel 1.25 to 2.25%; phosphorus and sulphur together, under .03%; manganese .45 to .65%; silicon .50 to 1.00%; carbon .35 to .45% and the principal part of the remainder iron.

- 5 2. Forged metal articles having high resistance to hot oxidation and composed of alloy steel containing chromium 7.00 to

GEORGE R. RICH.